

United States Patent  
Boose et al.

[15] 3,642,591

[45] Feb. 15, 1972

[54] ELECTRO ZINC PLATING SOLUTION

[72] Inventors: Cesar Adrianus Boose, The Hague; Maarten Johan Reidt, Voorburg, both of Netherlands

[73] Assignee: Nederlandse Organisatie Voor Toegepast-Natuurweten-Schappelijk Onderzoek Ten Behoeve Van Nijverheid Handel en Verkeer, The Hague, Netherlands

[22] Filed: Mar. 9, 1970

[21] Appl. No.: 17,978

[30] Foreign Application Priority Data

Mar. 11, 1969 Netherlands.....69/03711

[52] U.S. Cl. ....204/55 R

[51] Int. Cl. ....C23b 5/10, C23b 5/12, C23b 5/46

[58] Field of Search.....204/55 Y, 55 R, 43, 44, 114

[56]

References Cited

UNITED STATES PATENTS

3,298,938 1/1967 Shibasaki .....204/55 R

FOREIGN PATENTS OR APPLICATIONS

1,688 12/1902 Great Britain .....204/55

Primary Examiner—G. L. Kaplan

Attorney—Brumbaugh, Graves, Donohue and Raymond

[57]

ABSTRACT

A cyanide-free zinc plating bath is described. Besides a zinc salt in the usual concentration range and possible brighteners, it comprises a polyhydroxy acid or salt and boric acid and/or borate in a molar ratio of between about 1(zinc):1½(polyhydr oxy):3(boric) and 1:2:4, depending on the zinc content of the solution.

6 Claims, No Drawings

## ELECTRO ZINC PLATING SOLUTION

The invention relates to a solution and a method for electro zinc plating (galvanizing).

It is known that electrolytic zinc plating can be carried out in a cyanide solution. In addition to zinc and cyanide, such solutions usually contain auxiliary substances such as those which maintain the pH of the solution at a specific high value, which means acid or alkaline substances, as the case may be. Often included are also substances called brighteners, which are most aromatic aldehydes or derivatives thereof, either singly or mixed, or with substances of a different nature together forming the brightener. Examples are benzaldehyde, gelatin, 3,4-methylene-dioxy-benzaldehyde (piperonal), 4-hydroxy-3-methoxy-benzaldehyde (vanillin), 3,4-dimethoxy-benzaldehyde (veratraldehyde), protein decomposition products, and the like.

All such conventional additives can also be used within the scope of the present invention.

Prior to the electro zinc plating process taking place, the metal to be zinc plated is usually subjected to such pretreatments as degreasing. A common pretreatment is for instance degreasing in organic solvents, followed by degreasing in an alkaline medium, which may be carried out electrolytically, if necessary. After rinsing with water and pickling with hydrochloric acid, there is another rinsing with water. This is followed by the zinc plating process. After this, the metal is usually passivated. Examples of conventional passivating liquids are (all per litre of solution):

|                                        |                     |
|----------------------------------------|---------------------|
| CrO <sub>3</sub>                       | 30 g.               |
| H <sub>3</sub> PO <sub>4</sub> (pure)  | 10 cm. <sup>3</sup> |
| HCl (conc.)                            | 5 cm. <sup>3</sup>  |
| HNO <sub>3</sub> (conc.)               | 5 cm. <sup>3</sup>  |
| H <sub>2</sub> SO <sub>4</sub> (conc.) | 5 cm. <sup>3</sup>  |

or

|                                                |                    |
|------------------------------------------------|--------------------|
| Na <sub>2</sub> Cr <sub>2</sub> O <sub>7</sub> | 200 g.             |
| H <sub>2</sub> SO <sub>4</sub> (conc.)         | 6 cm. <sup>3</sup> |

With these conventional methods, the temperature is somewhere between 10° and 80° C. and the dipping time between 15 and 120 seconds. The material is passivated to give extra protection against corrosion and to provide a basis for a finish such as the application of a lacquer.

These preliminary and subsequent treatments are generally known techniques, and they can also be applied within the scope of the present invention.

There are objections against using cyanide solutions. It is particularly the high toxicity which gives rise to serious problems in removing spent solutions. Attempts have therefore been made for a very long time to use noncyanide solutions but in electro zinc plating cyanide solutions nevertheless still constitute a majority. Sometimes zincate solutions, which are based on the solubility of zinc salt in an alkaline medium, are used. Zincate solutions are expensive, however, and extremely sensitive to metal impurities.

Electro zinc plating is carried out mainly either in revolving drums or in stationary containers. In the first case the solution is automatically shaken, which is essential to prevent protracted inhomogeneities. A stationary solution can be agitated for instance by means of air.

The current density on the objects to be zinc plated is also according to the present method between about 0.1 and 10 amperes per dm.<sup>2</sup>; it is usually between about 3 and 6 amperes per dm.<sup>2</sup>.

The temperature is not so very important for the present method. The solution is an aqueous liquid, which means that it always remains above its solidification point and, for practical reasons, below its boiling point. In practice, the temperature will be somewhere between 20° and 80° C. It is true that at a higher temperature the electric conductivity of the solution increases and the efficiency improves, but at a lower temperature the brightness of the galvanized product is generally slightly better. The choice is therefore a matter of practice rather than theory.

Solutions are known which have a high or a low zinc content, each having its own specific advantages. Exactly the same applies to the solutions in accordance with the invention. An advantage of a solution with a high zinc content is that the cathodic current efficiency is higher than in a solution with a low zinc content; the latter has the advantages, however, of a slightly greater throwing power (see below) and cheaper waste water treatment.

Two terms are used in electro zinc plating.

“Variance” is used to indicate the following.

Assuming an object with many projecting and recessed corners, of which a common example is a metal screw bolt with its screw thread and the slot in its head for the screwdriver. Ideally, the applied zinc coat is equally thick everywhere; the degree of difference is referred to as variance.

“Cover” is used to indicate the following.

Assuming an iron cup has to be zinc plated. The cup is suspended in the solution and it is also filled with this liquid. In electroplating, ideally the inside bottom of the cup is also entirely covered with zinc; this effect is referred to as cover.

It is known that variance and cover are very much dependent on the composition of the solution.

It will be clear from the foregoing that all kinds of solution components and electroplating conditions are known, and all these conventional matters apply likewise to the present invention. Its essence is that the electroplating solution per litre of the bath must also contain 0.05 to 0.8 gram-atom zinc, a polyhydroxy acid or a salt thereof, as well as boric acid and/or borate. The molar ratio of zinc content and the polyhydroxy anion should be between about 1:1.3 and 1:2.2; the molar ratio of polyhydroxy anion to boric anion between about 1:1.8 and 1:2.2.

For the effect it makes no difference whatsoever whether polyhydroxy acid or a salt thereof is used and it is equally unimportant whether boric acid or borate is used. The choice is determined exclusively by factors beyond the scope of the invention, such as price, availability, keeping properties, and the like. It now appears advantageous to use sodium gluconate or sodium heptonate and boric acid, but this has nothing to do with the essence of the invention.

It is known that sometimes a low and sometimes a high zinc content has to be used. In practice a low zinc content is considered to exist in a solution with approximately 5 to 25 grams of zinc per litre, and a high zinc content in a solution with approximately 25 to 50 grams of zinc per litre.

For a low zinc content the three-component system, which forms the essence of the invention, appears to be best if made up of approximately 2 gram-molecules polyhydroxy acid or a salt thereof, and approximately 4 gram-molecules boric acid and/or borate per gram-atom zinc (10 percent deviation possible).

In solutions with a high zinc content, these ratios per gram-atom zinc are about at 1½ gram-molecule polyhydroxy acid or a salt thereof and 3 gram-molecules boric acid or borate (10 percent deviation possible).

At about 25 grams of zinc per litre ratios intermediary between the above-mentioned ratios may be used.

It has already been pointed out in the foregoing that the question whether polyhydroxy acids or salts thereof, or boric acid or borate are used, has nothing to do with the essence of the invention. This is all the more important because it is desirable to keep the pH of the solution between certain limits, which means in practice that free acids or free lyes are added. In this case dissociation equilibria occur, which make a difference between for instance boric acid and borate irrelevant. At all times the pH must be above 5; below this good results cannot be achieved with certainty. The upper limit depends on the composition of the solution. Particularly on the substance, mostly an inorganic salt such as sodium sulphate, which is present in the solution to increase the electric conductivity. With sulphates, the pH must not be raised beyond approximately 8, but with chlorides the limit may be higher. By means of a few tests, a specialist should be able to find the

correct pH, that is the pH at which, given the composition of the solution, the electro zinc plating process proceeds at an optimum level.

The zinc compound, which is always necessary in electro zinc plating baths, is usually and also according to the present method zinc sulphate or zinc chloride, but in view of the required pH it still makes no difference whether zinc sulphate and, for instance, sulphuric acid are added as pH controlling agents or another zinc compound such as ZnO, which in this case with H<sub>2</sub>SO<sub>4</sub> again brings zinc and sulphate ions into the solution anyway.

Ammonium ions should be avoided; they give less favorable results.

#### EXAMPLE I

A drum 30 cm. long and 15 cm. in diameter, with perforations totaling 6.7 percent, fitted with flexible contacts, contained 300 screw bolts with a total surface of 75 dm.<sup>2</sup>. The drum was placed in a zinc solution of 185 litres, which had the following composition per litre of solution:

|                                                   |      |       |
|---------------------------------------------------|------|-------|
| zinc<br>(as ZnSO <sub>4</sub> ·7H <sub>2</sub> O) | 16.5 | grams |
| sodium gluconate                                  | 110  | grams |
| boric acid                                        | 70   | grams |
| anhydrous sodium sulphate                         | 100  | grams |
| sodium hydroxide                                  | 13   | grams |
| benzaldehyde                                      | 0.2  | gram  |
| water                                             | 1    | liter |
| to make                                           |      |       |

The pH of the solution was 6.8. During galvanizing, the temperature remained between 50° and 60° C. The electroplating time was 1 hour at a current density of 1 ampere per dm.<sup>2</sup>. After this, the bolts were rinsed with water and put in a passivating solution, and finished. The efficiency was 75 percent.

As the benzaldehyde tends to become exhausted during electroplating, aldehyde was added after each drum charge in such a way as to maintain the aldehyde content at about 2 grams per litre.

#### EXAMPLE II.

Example I was repeated with a solution of the following composition per litre of solution:

|      |      |       |
|------|------|-------|
| zinc | 18.7 | grams |
|      | 45   |       |

(added as zinc chloride)  
boric acid  
sodium heptonate

91.5 grams  
150 grams

5 The pH was kept at 6.8, the temperature was 45° C. The charge was 15 kg. carriage bolts with a total surface of 165 dm.<sup>2</sup>; the electroplating time was 35 minutes, at a current density of 0.85 amperes per dm.<sup>2</sup>. The efficiency was 78 percent and the coat thickness of the zinc after passivating was 5.2 microns.

10 A remarkable advantage of these solutions is that with an amount of brightener (i.e., benzaldehyde) less than normal a gloss was obtained which was brighter than normal.

15 The cover of the objects zinc plated in accordance with the invention is excellent, and the throwing power of the solutions in accordance with the invention is good.

We claim:

1. An aqueous electroplating solution comprising about 0.05 to 0.8 gram-atom zinc per litre, polyhydroxy carboxylic acid or a salt thereof, and boric acid or borate, the molar ratio of zinc to polyhydroxy carboxylic acid or salt being from about 1:1.3 to about 1:2.2 and the molar ratio of polyhydroxy carboxylic acid or salt to boric acid or borate being from about 1:1.8 to about 1:2.2, the pH of the solution being at least about 5, and the solution being substantially free of ammonia.

25 2. An aqueous electroplating solution according to claim 1 comprising between 5 and 25 grams per litre zinc, about 2 gram-molecules polyhydroxy carboxylic acid or salt thereof per gram-atom zinc, and about 4 gram-molecules boric acid or borate per gram-atom zinc.

30 3. An aqueous electroplating solution according to claim 1 comprising between 25 and 50 grams per litre zinc, about 1.5 gram-molecules polyhydroxy carboxylic acid or salt thereof per gram-atom zinc, and about 3 gram-molecules boric acid or borate per gram-atom zinc.

35 4. An aqueous electroplating solution according to claim 1 containing from about 1.8 to 2.2 parts boric acid per part polyhydroxy carboxylic acid or salt thereof.

5. An aqueous electroplating solution according to claim 1 wherein the polyhydroxy carboxylic acid or salt thereof is sodium gluconate.

40 6. An aqueous electroplating solution according to claim 1 wherein the polyhydroxy carboxylic acid or salt thereof is sodium heptonate.

\* \* \* \* \*

UNITED STATES PATENT OFFICE  
CERTIFICATE OF CORRECTION

Patent No. 3,642,591 Dated February 15, 1972

Inventor(s) Cesar Adrianus Boose and Maarten Johan Reidt

It is certified that error appears in the above-identified patent and that said Letters Patent are hereby corrected as shown below:

First page, Item [73], line 3, after "Nijverheid" insert a comma. Column 1, line 10, "most" should be --mostly--. Column 3, line 45, "18.7 grams" should be --28.7 grams--.

Signed and sealed this 25th day of July 1972.

(SEAL)

Attest:

EDWARD M.FLETCHER, JR.  
Attesting Officer

ROBERT GOTTSCHALK  
Commissioner of Patents